

Nov. 14, 1961

61 E. A. GODAT, JR., ET AL 3,  
PROCESSING OF SELENIUM-CONTAINING METALLURGICAL  
DUSTS AND FUMES  
Filed April 15, 1959

3,008,806

BOSCH AND FOMES  
Filed April 15, 1959



INVENTORS  
J. B. QUINTANILLA, JR.  
and E. A. GOBAT  
BY *Harper T. Serjian*  
ATTORNEY

1

3,008,806  
PROCESSING OF SELENIUM-CONTAINING  
METALLURGICAL DUSTS AND FUMES

Edward A. Godat, Jr., and Joaquin B. Quintanilla, Monterrey, Nuevo Leon, Mexico, assignors to American Metal Climax, Inc., New York, N.Y., a corporation of New York

Filed Apr. 15, 1959, Ser. No. 806,652

9 Claims. (Cl. 23—209)

This invention relates to the processing of selenium-containing materials and relates more particularly to an improved process for upgrading the metallurgical dusts or fumes of low selenium content to a point where selenium recovery from such material is made economically practical.

The low selenium content of such materials renders impractical the application of the conventional procedures for selenium recovery therefrom utilizing for example, the well-known soda ash roasting process or selenium volatilization methods. For satisfactory results, such procedures require a feed material of appreciably higher selenium content than normally exists in the fumes or dust obtained from the gases produced in lead ore smelting or other metallurgical operations that result in production of a selenium-containing dust or fume. Accordingly, the low selenium content material must first be upgraded to increase the selenium concentration to a level that makes the processing for selenium recovery feasible. Satisfactory upgrading of dusts and fumes for the stated purpose is rather difficult to achieve in a completely satisfactory manner and because of this selenium recovery from such materials is not carried out resulting in the loss of the selenium values therein.

It is the principal object of this invention to provide an improved process for concentrating the selenium values in a low-grade metallurgical dust or fume to enable the subsequent recovery of said selenium in an economic and practicable manner.

It is another object of this invention to provide an improved process for concentrating the selenium content in a metallurgical dust or fume by flotation methods.

Other objects and advantages will become readily apparent as this specification proceeds.

We have now discovered that upon subjecting metallurgical dusts and fumes of relatively low selenium content to a densification roast and thereafter grinding the roasted material and extracting the water-solubles therefrom, the residual material, upon appropriate conditioning, and flotation provides a selenium concentrate having a significantly increased selenium content. The flotation product being at least ten times richer in selenium than the original metallurgical dust or fume provides an excellent feed material for use in the well known selenium recovery procedures.

The metallurgical fumes and dusts referred to herein are of a varied type and character wherein the selenium content of the material generally ranges from 1 to 5% by weight or possibly slightly higher. A principal source of such material is the lead blast furnace dust collected, for example, in an electrostatic precipitator. Although the treatment of such material is hereinafter described more fully for purpose of illustration, it will be understood that the invention is not limited thereto but is also applicable to other low grade metallurgical dusts and fumes typically containing around 1 to 5% selenium.

In a preferred embodiment of the invention, the dust and fume from a lead blast furnace collected by means of a Cottrell precipitator or other collecting apparatus is removed for treatment in accordance with the present invention. Initially, the material is subjected to a densifying roast which is effective for converting the light,

2

fluffy amorphous material to a more crystalline or denser form to make it more amenable for subsequent treatment. This is accomplished by heating said material in any suitable furnace such as a muffle or hearth roaster to a temperature between 200 and 500° C. for a period ranging from about 10 minutes to an hour or so depending on the temperature actually used with a period of about 20 minutes sufficing at the preferred roasting temperature of about 300° C. Air need not be excluded during the densifying roasting.

The densified material is then ground in a ball mill or by any other appropriate means for producing material of suitable particle size preparatory to treatment thereof by froth flotation. In this connection, a grind in which about 85% of the material is reduced to minus 200-mesh screen size has been found to produce satisfactory flotation recoveries. Prior to actual flotation, however, it is essential that the densified material be leached with water to remove the soluble salts contained therein.

The step of grinding the material and then extracting with water for the removal of water-solubles may be carried out more or less simultaneously as by resorting to wet grinding wherein the water for leaching the material is added directly to the ball mill during the grinding operation. The slurry obtained thereby upon completion of the grinding may then be filtered or centrifuged to separate the aqueous liquid containing the water-solubles from the selenium-containing residue. The amount of water used for leaching the comminuted material is not of particular significance, it being important, however, to extract the water-soluble salts as completely as possible using several washes if necessary.

Alternatively, the densified smelter dust or fume may be leached prior to grinding with the leached calcine being then ground preparatory to its being subjected to flotation. For best results, however, it is preferred to leach the material in a comminuted state since the extraction of the water-soluble salts is made easier and more effective thereby. In actual practice, the leaching operation is best effected by a combination of both approaches in that the calcine obtained from the densifying roast may be leached to remove a major portion of the water-soluble constituents, the remainder being thereafter extracted during comminution of the material in the presence of water as previously mentioned. In either event, the material substantially freed of its water-soluble constituents should be made available for pulping and ensuing flotation in a form suitable for the purpose.

That the prior treatment of smelter dusts and fumes of low selenium content is essential for enabling successful flotation for the purpose of obtaining a satisfactory selenium concentrate product is made readily apparent by comparative tests on batches of the same feed material. For example, all tests on raw dusts and fumes referring to attempts to obtain a satisfactory selenium flotation concentrates were negative as were the results using material that was densified but not leached prior to flotation. By contrast, results on leached densified smelter dusts and fumes proved exceedingly satisfactory in that the subsequent flotation as will be herein-after described in detail produced highly satisfactory results.

The effect of the densifying roasting and leaching on smelter dusts and fumes is illustrated in the case of Cottrell dust from lead blast furnacing wherein, for example, a 2500 gm. sample assaying 1.25% by weight of selenium was densified at 250° C. for one hour in a gas fired furnace to yield 2040 gm. of calcine still assaying 1.25% selenium. The calcine, after leaching with water yielded 1700 gm. of residue assaying 1.5% selenium.

The residue was ground for 10 minutes in a steel ball mill with seven liters of water. Even without separating the water at this stage the resulting pulp produced by the aforesaid grinding gave very good flotation results whereas in the absence of either the densifying roasting or the leaching steps the flotation results were negative.

Following removal of substantially all of the water-soluble content from the calcined material preferably while in a ground state, the residue is treated to provide 10 an aqueous pulp for use in froth flotation. It has been found that froth flotation is best carried out on a conditioned aqueous pulp containing from 20 to 40% and preferably about 30% solids, the mixture being made 15 slightly acidic by the addition of sulfuric acid to provide a pH between 5.0 and 6.8 and preferably about 6.0. At appreciably lower pH values, the recovery of selenium has been found to be materially reduced. It has also been found that the conditioning period of the reagentized pulp prior to actual flotation also materially affects the 20 results obtained depending somewhat on the nature of the material being processed. Conditioning periods of from 5 to 30 minutes generally are satisfactory in the usual case, after which a frother reagent is added if omitted during the conditioning step. Thereafter, flotation 25 is carried out in the usual manner in any desired type of conventional froth flotation cell.

Although collectors and frothers commonly used in froth flotation concentration of metalliferous ores may be used for obtaining the desired selenium concentrate product, with the collector reagents generally consisting of amines, fatty acids, xanthates and the like and the frother reagents consisting of substances such as pine oil, alcohols, phenols, cresols, glycols, glycol ethers and the like, it has been found that a xanthate collector used 30 in the amount of about 0.05 to 0.50 lb. per ton of leached residue feed and glycol ether type frother used in the amount of about 0.05 to 0.20 lb. per ton of leached residue feed provide the best results. Of the xanthates which are commonly used in the form of alkali metal 35 salts including substances such as sodium ethyl xanthate, potassium amyl xanthate, sodium hexyl xanthate, sodium amyl xanthate and the like, the product potassium hexyl xanthate known commercially as Z-10 has proven to be very effective as a collector reagent. In some instances, the consumption of collector reagent may be decreased 40 and the recovery of selenium in the concentrate increased somewhat by using kerosene or an equivalent substance in conjunction with the xanthate collector reagent. With respect to the frother reagents, the product known commercially as Dowfroth 250 which is understood to be a polypropylene glycol ether has been found to be highly satisfactory.

The flotation of the conditioned pulp is carried out in an entirely conventional manner with the frother being added in the indicated proportion either to the conditioner or upon introduction of the conditioned pulp to the flotation cells. Flotation may be carried out in as many stages as desired but usually one cleaning of the rougher concentrate without additional reagents suffices to give a desirable product without incurring undue losses of selenium to middlings. The froth product from the cells generally contains from about 12 to 20% by weight of selenium, the recovery of selenium usually amounting to better than 60%. Cadmium, if present in the feed material, is also recovered as a component of the concentrate product in amounts corresponding to better than 50-60% of the quantity present in the leached residues. A representative concentrate product obtained from lead blast furnace dusts and fumes assaying 1.6% by weight of selenium and 2.6% by weight of cadmium after roasting and leaching assayed at 16% selenium and 24.6% cadmium following froth flotation as hereinbefore described.

The process comprising the present invention as discussed above is illustrated in the accompanying drawing

wherein the various operations are schematically indicated. Although the grinding and leaching steps are shown as separate and distinct steps in the flow sheet, it will be understood these steps can be combined in one 5 operation as previously stated.

While in the foregoing specification this invention has been described in relation to a preferred embodiment thereof and specific details of this embodiment have been set forth for the purpose of illustration, it will be apparent to those skilled in the art that this invention is susceptible to other embodiments and that many of the details herein set forth can be varied considerably without departing from the basic concept of the invention.

What is claimed is:

1. In a process for the recovery of a selenium concentrate from metallurgical dusts and fumes containing selenium in relatively small quantities generally below 5% by weight, the steps comprising roasting said dusts and fumes to provide a densified calcine, grinding said calcine, leaching the ground calcine with water to remove substantially all the water-soluble content therefrom, pulping said ground and leached residue in water, acidifying the resulting mixture to a pH between 5.0 and 6.8, reagentizing and conditioning the mixture, subjecting the conditioned mixture to froth flotation and recovering a selenium-enriched fraction therefrom.

2. The process of claim 1 wherein the roasting operation is carried out at a temperature of about 300° to 450° C. for a period of about 20 minutes.

3. The process of claim 1 wherein prior to froth flotation the ground and leached residue is pulped in water to a solids content from about 25 to 35%.

4. In a process for the recovery of a selenium concentrate from metallurgical dusts and fumes containing selenium in relatively small quantities generally below 5% by weight, the steps comprising roasting said dusts and fumes to provide a densified calcine, leaching said calcine to remove water-soluble materials therefrom, grinding the leached residue, pulping the ground and leached residue in water, acidifying the resulting mixture to a pH between 5.0 and 6.8, reagentizing and conditioning the mixture, subjecting the conditioned mixture to froth flotation and recovering a selenium-enriched fraction therefrom.

5. The process of concentrating the selenium contained in a metallurgical dust from smelting of lead ores, said dust generally containing below 5% by weight of selenium comprising the steps of roasting said dust for from 10 minutes to an hour at a temperature ranging from 200 to 450° C., grinding the resulting calcine, leaching the ground material with water to effect removal of at least a major portion of the water-soluble content therefrom, pulping the resulting ground residue in an aqueous medium to a solids content of from 25 to 35% said aqueous medium being acidified to a pH between 5.0 and 6.8, reagentizing the acidified aqueous pulp with a xanthate collector, conditioning the reagentized pulp for from 10 to 30 minutes, subjecting the conditioned pulp in the presence of a frother reagent to flotation and recovering a selenium-enriched concentrate.

6. The process of claim 5 wherein the grinding and leaching steps are carried on simultaneously.

7. The process of claim 5 wherein the frother reagent is a polypropylene glycol ether.

8. The process of claim 5 wherein the xanthate collector is potassium hexyl xanthate.

9. The process of claim 5 wherein kerosene is used in conjunction with the xanthate collector.

References Cited in the file of this patent

70 Gmelin: "Handbuch der anorganischen Chemie," System No. 10, Selenium, 8th ed., 1949, pages 78-95, page 86 especially relied on.

J. Perry's "Chemical Engineers Handbook," 3rd ed., McGraw-Hill Book Co., Inc., New York, N.Y., 1950, page 1088.